

Patented July 18, 1939

2,166,496

# UNITED STATES PATENT OFFICE

2,166,496

## ALUMINUM ALLOYS

Isamu Igarashi and Goro Kitahara, Fuse, Japan,  
assignors to Sumitomo Kinzoku-Kogyo Kabu-  
shiki Kaisha, Osaka, Japan

No Drawing. Original application June 20, 1938,  
Serial No. 214,809. Divided and this applica-  
tion April 6, 1939, Serial No. 266,419. In Japan  
December 15, 1936

1 Claim. (CL 75—142)

This application is a division of the applicants' earlier application, Ser. No. 214,809, filed June 20, 1938.

This invention relates to improved light alloys having high tensile strength and consisting of zinc, copper, magnesium, manganese, chromium, calcium and aluminum, and has for its object to provide light alloys devoid of season cracking.

Hitherto, such light alloys as E alloys and Sander's alloys which consist of copper, zinc, magnesium, manganese and aluminum have been known as having high tensile strength; but where

24 hours. Then they were bent so that the inner surface of both ends of the strips met, and they were tied up with wires at points 20 mm. from each end, and were left alone, special attention being paid to the middle part of the strips to see whether or not cracks would appear in the course of time. 5

The results of the above-mentioned experiments, the compositions of the test pieces used, namely, E alloy, Sander's alloy and some representative alloys according to the present invention, are presented in the following table: 10

| 15 | No. | Composition, percent |    |     |     |      |      |    | Tensile strength<br>Kg/mm. <sup>2</sup> | Elongation<br>at 50 mm.<br>Percent | Crack          | 15                                           |    |
|----|-----|----------------------|----|-----|-----|------|------|----|-----------------------------------------|------------------------------------|----------------|----------------------------------------------|----|
|    |     | Cu                   | Zn | Mg  | Mn  | Ca   | Cr   | Al |                                         |                                    |                |                                              |    |
| 20 | 1   | 2.5                  | 20 | 0.5 | 0.5 | —    | —    | —  | Rest<br>do                              | 60<br>55<br>59                     | 10<br>15<br>14 | Appears within one day.<br>Do.<br>Do.        | 20 |
|    | 2   | —                    | 8  | 1.5 | 0.5 | —    | —    | —  | do                                      | 59.6                               | 15             | No appearance even after<br>one year.<br>Do. |    |
|    | 3   | 2                    | 8  | 1.5 | 0.5 | —    | —    | —  | do                                      | 61.0                               | 14             | Do.                                          |    |
|    | 4   | 2                    | 8  | 1.5 | 1.2 | 0.02 | 0.02 | —  | do                                      | 60.0                               | 14             | Do.                                          |    |
|    | 5   | 2                    | 8  | 1.5 | 1.5 | 0.04 | 0.25 | —  | do                                      | 59.8                               | 15             | Do.                                          |    |
|    | 6   | 2.5                  | 10 | 1.5 | 1.5 | 0.05 | 0.25 | —  | do                                      | 60.0                               | 14             | Do.                                          |    |
|    | 7   | 2                    | 8  | 1.5 | 0.5 | 0.03 | 0.30 | —  | do                                      | 59.8                               | 15             | Do.                                          |    |

25 the utmost strength and durability are required, they were unsuitable for use due to their harmful property of season cracking. The present invention accordingly is to obviate the above-mentioned defect and to provide an alloy which is well adapted for use where non-season cracking is essential.

After a long series of tests and investigation, it was discovered that the addition of 0.05-1% of chromium and 0.01-0.2% of calcium to the known alloys was effective in eliminating from the alloys the defect of season cracking without sacrificing their tensile strength. Moreover, these elements are capable of making the grain structure of the alloys in the cast state much finer and consequently impart forgeability thereto. These elements also have a tendency to increase the fluidity of the molten metal in the refining process. Still further, the presence of not more than 1% of iron or silicon as impurities does not impart any inferior quality to the alloys. The present invention accordingly provides aluminum alloys containing 1-3% of copper, 4-20% of zinc, 1-2% of magnesium, 0.1-2% of manganese, 0.01-0.5% of chromium, 0.01-0.2% of calcium, and less than 1% of iron and silicon as impurities.

55 Test pieces which had been properly quenched and tempered were subjected to tensile tests and the season cracking test, these tests being conducted with utmost care. Strips of 1 mm. in thickness, 2 mm. in width, and 200 mm. in length, made of many different aluminum alloys were hardened by heating them up to 450° C. and suddenly cooled in water. After this, they were annealed at a temperature of 125° C. for about

25 Pieces 1 and 2 in the above table represent the light alloys widely known as E alloy and Sander's alloy, respectively. Piece 3 is about the same in the range of constituents and composition as Nos. 4 to 7, but lacks the chromium and calcium content. Pieces 4 to 7 are alloys made according to the present invention.

30 It is clear from the foregoing table that an addition of a small percentage of chromium and calcium to the alloys imparts to them forgeability and a remarkable resistance to season cracking. 35 The light alloys of the present invention are therefore peculiarly well suited for use in many situations where high tensile strength and non-season cracking are essential, as in the case of 40 materials for aeroplane manufacturing.

45 In making the alloys according to this invention, three different mother alloys consisting of aluminum and copper, of aluminum and manganese, and of aluminum and chromium are first prepared, and these three alloys are then melted together with aluminum, to which magnesium and zinc are further added. Experiments show that an addition of 0.01 to 0.5% of titanium to the alloys increases the quality of the alloys 50 to a large extent.

55 Having described the invention, what is claimed is:

Aluminum alloys characterized by ready forgeability and resistance to season cracking and consisting of 4-20% of zinc, 1-3% of copper, 1-2% of magnesium, 0.1-1.5% of manganese, 0.05-1% of chromium, 0.01-0.2% of calcium, and the rest of aluminum.

ISAMU IGARASHI.  
GORO KITAHARA. 60